

Patented Feb. 1, 1927.

1,616,364

# UNITED STATES PATENT OFFICE.

HOWARD M. GERMAN, OF CRAFTON, PENNSYLVANIA, ASSIGNOR TO UNIVERSAL STEEL COMPANY, OF BRIDGEVILLE, PENNSYLVANIA, A CORPORATION OF PENNSYLVANIA.

## HACK SAW.

No Drawing.

Application filed April 19, 1926. Serial No. 103,148.

The present invention relates to hacksaws and especially to the finished hacksaws, the steel from which they are made and the process of treating the steel.

5 Hacksaw steel as made at the present time is practically a standard article and has approximately the following composition:—

|             |              |
|-------------|--------------|
| Carbon      | 1.00 to 1.40 |
| Manganese   | .20 to .40   |
| 10 Silicon  | .10 to .30   |
| Sulphur     | .02 maximum  |
| Phosphorus  | .02 maximum  |
| Tungsten    | 1.00 to 2.00 |
| 15 Chromium | .00 to .25   |

15 The steel is rolled into sheets of varying thicknesses from the ingots or billets. The sheets after finishing on a sheet mill are "floor annealed" by reheating to temperatures of 1000 to 1250° F., after which they are laid on top of previously worked sheets. The sheets are thus cooled in pack form, which retards the cooling somewhat.

20 The floor annealing removes strains and 25 renders the material sufficiently soft for shearing, milling and setting operations for producing the finished hacksaw. The steel in the annealed sheet form has a metallographic structure consisting principally of sorbite, cementite and probably smaller amounts of pearlite. The cementite exists in the form of finely divided particles or patches uniformly distributed through the steel and drawn out into elongated shape or 30 lines by the rolling of the sheets. The particles of cementite are too fine to have any useful or appreciable action as abrasive grains in the steel. The cementite lines cause planes of weakness and brittleness in the 35 steel which are not materially changed or altered by the annealing and hardening treatment ordinarily practiced.

40 The hacksaws as fabricated from the sheets are then hardened. It has been the aim in the 45 hardening of hacksaws to produce as uniform a structure as possible, it being the belief that the more uniform structure would give the best cutting results. The hardening has, therefore, been carried out by heating the 50 saw blades to a temperature well above the critical point, and holding for a time sufficient to not only convert the sorbite into

martensite and austenite, but also to take the cementite into solution and then quickly quenching in oil. After hardening, the 55 blades are tempered to produce a structure of martensite with varying amounts of troostite and sorbite. The resultant steel in the finished hacksaw blade has, therefore, been almost wholly martensite with varying 60 amounts of troostite and sorbite, and with little or no free cementite.

I have discovered that the cutting and wearing qualities of hacksaws may be greatly improved by having free cementite in the 65 form of nodules in the finished hacksaw. The metallographic structure of the finished hacksaw consists of hard abrasive particles of cementite embedded in a softer and tougher matrix, usually martensite with varying 70 amounts of troostite and sorbite. As is well known, the cementite or free carbide is very hard, in fact, being the hardest constituent of steel.

The advantages of having the steel structure containing the hard cementite nodules 75 will be apparent from consideration of the action of the hacksaw in cutting. When the hacksaw first starts to cut, the sharp cutting points of the teeth remove a curled chip 80 somewhat similar to the action of a lathe tool. After the hacksaw teeth become dull and slightly rounded, curled chips are no longer produced. Unlike other metal cutting saws and tools, the teeth of a hacksaw 85 are not ground or sharpened on becoming dull, but the saw is allowed to operate until it is worn out. After the teeth become dull so as to no longer be capable of cutting curled chips, a considerable portion of the 90 cutting is dependent upon the abrasive property of the steel.

I have found that the hard nodules of cementite in my improved hacksaw give the 95 hacksaw a much greater abrasive property than hacksaw blades having the usual uniform metal structure. As a result, my hacksaw blades have been found to do from 50% to 300% more work than the usual hacksaws. In addition to cutting considerably better, the matrix or bond of my hacksaws is decidedly tougher, and the saws are less liable to break.

By the process of heat treatment herein-

after described, I have been able to utilize the ordinary hacksaw steel of a composition described above, although I prefer to vary this composition somewhat by increasing its 5 tungsten and chromium content.

The process will first be described in connection with the usual hacksaw steel, the analysis of which is described above.

After the sheets are finished on a sheet 10 mill in the usual way, they are given a special annealing treatment, which causes the cementite to coalesce into the desired abrasive nodules instead of being uniformly distributed in the patches or lines as in the usual 15 annealing treatment.

My special annealing treatment consists 20 in packing the steel sheets in an annealing box to exclude air and furnace gases, and heating to a temperature slightly under the critical point, and then slowly cooling. With the usual hacksaw steels, the annealing 25 temperature is about 1350° to 1375° F. The sheets are heated at this temperature for about eighteen hours and are then allowed to slowly cool in the furnace, as is the usual 30 practice in annealing, for about thirty hours. This special annealing at the higher annealing temperatures causes the free cementite to be converted from its more or less uniform 35 patch or line-like distribution, into small nodules or spheroids of a size to serve as abrasive grains in the finished saw. The structure of the steel after annealing is principally sorbite, with probably small 40 amounts of pearlite, in the form of a matrix holding the embedded nodules of cementite. The annealed sheets are then subjected to the usual shearing, milling and setting operations to form the hacksaw blades.

The blades are then hardened. My hardening treatment differs radically from that 45 now employed in that instead of heat treating to form a uniform martensitic-austenitic structure, a non-uniform or heterogeneous structure is formed by preserving the cementite in its nodular form produced during the annealing operation. The hardening is 50 accomplished by heating the hacksaw blades to just over the critical point, usually about 55 50° to 100° F. above the critical point, and quenching.

The blades are brought up to this temperature and held there for two or three minutes, and then immediately quenched in oil. The 60 temperature and time of heating should be such as to take the sorbitic matrix into solution, but without dissolving any appreciable amounts of the nodular cementite. The steel after quenching, consists of a ground mass or matrix of martensite with a considerable amount of free cementite in the form of nodules or grains disseminated through the matrix.

Tempering, which is also done to produce a tougher saw blade, changes some of the

martensite to troostite and sorbite, but does not alter the cementite nodules which have been preserved through the hardening treatment.

While hacksaw blades having improved 70 cutting and wearing qualities may be produced by my process from the present day standard hacksaw steel, I have found that still better hacksaw blades may be produced by varying the standard composition somewhat and treating it by the same process as 75 that described above. In modifying standard hacksaw steel formula, I increase the tungsten and chromium because the tungsten and chromium increases the quantity of the 80 hard segregated cementite nodules in the finished saws.

The preferred composition of the steel is carbon .90 to 1.50%, preferably 1.10 to 1.40%, tungsten preferably 2.00 to 5%, but 85 not over about 7%, chromium preferably .50 to 2.50% but not over about 3%, and manganese, silicon, sulphur and phosphorus within the usual ranges of crucible and tool steels, the manganese being preferably .20 to .50%, 90 silicon preferably .15 to .30%, and the sulphur and phosphorus preferably not over about .04% each. This steel can be made and rolled about the same as the usual standard present day hacksaw steel. Its chromium, 95 and particularly its tungsten content, is much less than the more expensive high speed steel and is to be distinguished from high speed steel.

The increased chromium and tungsten 100 serve to increase the amount of cementite formed into the abrasive nodules and, therefore, produces a hacksaw blade superior to that made by my process from the lower tungsten and chromium standard hacksaw 105 steel formula. The increased quantities of tungsten and chromium, in addition to increasing the abrasive properties of the steel, also act as a brake to prevent the transition of the martensitic matrix to the softer 110 troostite and sorbite, thus resisting the tempering of the matrix by the frictional heat generated in cutting.

In describing the hard carbide or carbides forming the abrasive nodules, I have described them as cementite, using the term as one of general definition and not of limitation, and all to include not only the pure iron carbide, but also the impure cementite containing tungsten and chromium carbides in 115 combination with the iron carbide. Such free cementite is often referred to as carbides or free carbides.

While I have specifically described the preferred embodiment of my invention, it is 120 to be understood that the invention is not so limited, but may be otherwise embodied within the scope of my claims.

I claim—

1. A hardened steel hacksaw blade con- 130

containing embedded nodules of coalesced cementite of a size sufficient to serve as abrasive grains.

2. A hardened steel hacksaw blade containing tungsten not over about 7%, and containing embedded nodules of cementite of a size sufficient to serve as abrasive grains.

3. A hardened steel hacksaw blade containing between about 1% to 7% tungsten and chromium not over about 3% and containing embedded abrasive nodules of cementite.

4. A hardened steel hacksaw blade containing about 2% to 5% tungsten and about 15 .5% to 2.5% chromium and containing embedded abrasive nodules of cementite.

5. A hardened steel hacksaw blade containing tungsten not over about 7% and having a metal structure characterized by free 20 cementite segregated in nodular form in a matrix of softer metal, said nodules of cementite being of a size sufficient to serve as abrasive grains.

6. As an intermediate product in the manufacture of steel hacksaw blades, an annealed steel sheet containing embedded abrasive nodules of cementite.

7. As an intermediate product in the manufacture of steel hacksaw blades, an annealed 30 steel sheet containing tungsten not over about 7%, and containing embedded abrasive nodules of cementite.

8. As an intermediate product in the manufacture of steel hacksaw blades, an annealed 35 steel sheet containing between about 1% and 7% tungsten, and chromium not over about 3%, and containing embedded abrasive nodules of cementite.

9. As an intermediate product in the manufacture of steel hacksaw blades, an annealed 40 steel sheet containing about 2% to 3% tungsten and about .5% to 2.5% chromium, and containing embedded abrasive nodules of cementite.

10. The process of hardening hacksaw 45 blades of steel containing abrasive nodules of cementite, which comprises heating them to a temperature and for a time sufficient to cause the steel matrix to go into solution but insufficient to permit the dissolution of 50 appreciable amounts of the cementite nodules, and quenching.

11. The process of hardening hacksaw 55 blades of steel containing embedded abrasive nodules of free cementite, which comprises heating them to a temperature of just over the critical point for a time insufficient to cause the cementite nodules to go into solution and quenching.

12. The process of making steel hacksaws 60 which comprises forming into sheets a hacksaw steel containing free cementite, annealing the sheets so as to cause the cementite to coalesce into nodules, fabricating hacksaw blades from the sheets, and hardening the 65 blades by heating them to a hardening temperature and for a time insufficient to break up the cementite nodules, and quenching.

13. The process of making steel hacksaws which comprises making a hacksaw 70 steel containing tungsten not over about 7% and chromium not over about 3% and characterized by the presence of free cementite, forming the steel into sheets, annealing the sheets by heating to a temperature below that 75 at which the cementite goes into solution but sufficient to cause the cementite to coalesce into nodules, fabricating hacksaw blades from the annealed sheets, and hardening the 80 blades by heating to a temperature and for a time sufficient to cause hardening after quenching but insufficient to cause the cementite nodules to go into solution to a substantial extent, and quenching.

In testimony whereof I have hereunto set 85 my hand.

HOWARD M. GERMAN.